

## UNITED STATES PATENT OFFICE

1,964,791

## PROCESS OF MAKING SAFETY PAPER

Frank S. Wood, Quincy, Mass.

No Drawing. Application July 22, 1931,  
Serial No. 552,550

1 Claim. (Cl. 91—67.95)

By bi-functional step is meant of or belonging to two proper offices or works of an agent which, in the manufacture of paper, has heretofore had but one office. For example, the office of a size-  
5 tub is to size the paper. By adding to it the office of chemically treating the paper with the same operation as the sizing, the liquid mixture is given two functions; my invention gives it a double action of an entirely different nature  
10 which is therefore a bi-functional step in the paper making process.

This invention relates to so called safety papers and to the processes of making such papers so that when written on with ink, the writing  
15 cannot be removed, altered or replaced without setting the ink in such writing or leaving tell-tale stains, discolorations or alterations visible on the surfaces of such paper, or both.

Its salient purpose is to provide an alternative  
20 step or improvement in a process of making safety paper by one continuous operation over that for which my application for a patent was filed November 8, 1930, Serial Number 494,443. Its other purpose is for an improved bi-func-  
25 tional step in other processes of making safety papers that are not one continuous operation.

The novelty consists in the simultaneous application to a web of paper of a chemical inkset composition made up of ferrocyanide of potassium dissolved in water so as to give a moderate alkalinity to a normally acid paper and varying in proportions with different grades and colors of paper but having a delicate balance which not only im-  
30 pregnates the paper with inksetting power but also sizes the paper to the degree required for a good writing surface. For further details, see my specification for a safety paper filed Apr. 22, 1931, Ser. No. 532,115. When, however, this sur-  
35 face is written upon with ink and a prolonged application of chlorine has been made for the purpose of bleaching the ink, then the delicate balance is evidenced by the fact that the chlorine dissolves or breaks down the sizing and the paper is ruined for writing purposes for the reasons  
40 that it not only spoils the surface of the paper and makes the ink feather but it also changes the color of the same re-written ink, thus fur-  
45 nishing obvious and various means of detecting that the writing has been tampered with. In combination with another liquid tub sizing application necessary or desirable in the fabri-  
50 cation of paper, in the surface coloring of paper, either or both. Tub-size is made of starch, glue  
55 and wax, at present; other materials may here-

after be adapted to sizing; my chemical solution is adaptable to each; my invention comprehends the use of any chemical solution with tub-sizing that would result in producing inkset safety paper by means of a bi-functional step. Such simultaneous application performs a double function at the mechanical cost of a single application, avoids the substantial costs of rehandling, re-processing, refinishing and rewinding. It also produces a better inkset than has heretofore been obtained by other methods including expensive machines for chemically treating the paper.

It is well known that the sizing of paper produces a sort of delicate layer of varnish upon its surface that results in the desired writing finish. I have discovered that by using a given proportion of my inkset liquid in place of that same proportion of water in the sizing, the sizing solution is not injured. Therefore, by mixing my inkset liquid which is a chemical composition with the sizing, in the application of this mixture, the paper absorbs both the sizing and the inksetting liquid at one and the same operation.

I have also discovered that by using a given proportion of my inkset liquid in place of the same amount of water in the mixing of dyes or so called fugitive ink, the dyes are not injured. Therefore, by mixing my inkset liquid with the dye which is to be applied to white paper for the purpose of coloring its surfaces, the paper is also impregnated with my inkset composition at one and the same operation.

Both discoveries constitute a bi-functional step in the process of manufacturing either a white safety paper as it is being run through a paper-making machine, or a colored safety paper of the La Monte or Hammermill type at the same time that the tint and design is being applied to the surfaces of the latter. This obviates the necessity of installing a separate machine for applying the inkset treatment to the web of paper either as a continuous or a rehandling operation.

I will first describe the application of my invention to the making of safety paper by one continuous operation. The paper as it is being made on the Fourdrinier machine is dried out and, while hot, is taken down into a tub under a roll immersed in a liquid mixture composed of sizing and inkset solution kept at a desired constant temperature; the hot, porous paper absorbs enough of the sizing to supply the proper writing surface and at the same time absorbs enough of the inkset solution mixed with the sizing to give the paper the power of setting ink written on its surface when ink eradicator is applied for

the purpose of removing the writing. Then the paper goes to other drying rolls, thence to the calender where it is finished and thence to the reel where it is wound up as safety paper, at one 5 continuous operation.

In the application of my invention to the other type of safety paper process, when the web of paper is run through a suitable container filled to its desired level with colored water mixed with 10 a predetermined amount of my inkset solution, the paper absorbs the moisture of the liquid mixture, colors both surfaces of the web of paper and passes on between rolls that utilize the tint to impress some form of design upon the 15 surfaces of the paper; while this is taking place, the paper is also absorbing inkset solution. Then, the paper is dried by whatever method is in use at that particular plant and is ready to be rewound into reels or to proceed to the cutting 20 machines, according to the system prevailing.

For the purpose of my present invention it is not believed to be necessary to set forth either the many formulas for giving the inkset feature to innumerable grades and makes of paper that 25 vary accordingly as well as with different colors and makes of dyes. It is obvious that these are almost infinite for the reason that the same grade of paper made at a different mill requires a different formula, and each different grade as 30 well. Again a 10% inkset solution of a given strength in 90% of sizing or colored water may be made equal to another 20% solution by using double the quantity of chemicals for the same volume of inkset solution. I have taken this up 35 in specific instances in other preceding pending patents. A proper balance of the mixture may be had either by keeping the sizing constant in strength and varying the proportions of the

chemical inkset solution until the desired attributes are obtained in a given make or grade of paper, or by increasing or decreasing the strength of the chemical solutions without changing their proportions. Again, the strength of the sizing 80 may be increased or decreased as well as the variation in proportions; and it may be found desirable, in certain kinds of paper, to do both.

One of the formulas which I have used with good results calls for a unit volume of mixture composed of 80% sizing and 20% chemical solutions. I have had an equally good result by using 50% colored water and 50% chemical solutions. Various proportions of inkset solutions must necessarily be employed, for dyes vary in strength 85 both as to color and make; and, regardless of color, the same grade of white paper made by different manufacturers, requires different formulas. Therefore, it is clear that the variations in papers themselves, in their sizing and in their 90 dyes, demand various proportions in the amount and strength of inkset or chemical solutions without departing from the spirit of my invention.

What I therefore claim and desire to secure by 100 Letters Patent is:

In a process for making safety paper by one continuous operation, a bi-functional step comprising ink set solutions and sizing in such proportions that the ink setting chemicals do not 105 interfere with the proper sizing of the paper, and the sizing does not interfere with the transmuting of ordinary paper into safety paper when both sizing and ink setting solutions are mixed together and applied to a web of hot, dry paper 110 in the same bi-functional step, and without changing the normal color of the paper.

FRANK S. WOOD.

40

115

45

120

50

125

55

130

60

135

65

140

70

145

75

150